



US005998106A

# United States Patent [19]

Merkel et al.

[11] Patent Number: 5,998,106

[45] Date of Patent: Dec. 7, 1999

[54] **PHOTOGRAPHIC ELEMENT CONTAINING CYLACETAMIDO YELLOW DYE-FORMING COUPLERS**

[75] Inventors: **Paul B. Merkel**, Victor; **David A. Steele**, Webster; **Jerrold N. Poslusny**, Rochester; **Thomas R. Welter**, Webster, all of N.Y.

[73] Assignee: **Eastman Kodak Company**, Rochester, N.Y.

[21] Appl. No.: 09/069,391

[22] Filed: **Apr. 29, 1998**

[51] Int. Cl.<sup>6</sup> ..... **G03C 7/46**

[52] U.S. Cl. ..... **430/389**; 430/557; 430/544

[58] Field of Search ..... 430/388, 389, 430/556, 557, 544

## [56] References Cited

### U.S. PATENT DOCUMENTS

|           |         |                  |       |         |
|-----------|---------|------------------|-------|---------|
| 3,933,500 | 1/1976  | Shiba et al.     | ..... | 430/505 |
| 5,213,958 | 5/1993  | Motoki et al.    | ..... | 430/557 |
| 5,314,797 | 5/1994  | Yoshioka et al.  | ..... | 430/546 |
| 5,338,651 | 8/1994  | Naruse et al.    | ..... | 430/557 |
| 5,362,617 | 11/1994 | Morigaki et al.  | ..... | 430/557 |
| 5,374,507 | 12/1994 | Yoshioka         | ..... | 430/557 |
| 5,612,174 | 3/1997  | Takizawa et al.  | ..... | 430/557 |
| 5,674,667 | 10/1997 | Clark et al.     | ..... | 430/557 |
| 5,719,018 | 2/1998  | Katsumata et al. | ..... | 430/557 |

### FOREIGN PATENT DOCUMENTS

|         |        |         |
|---------|--------|---------|
| 5005974 | 2/1990 | Japan . |
| 2109P98 | 9/1991 | Japan . |

Primary Examiner—Geraldine Letscher  
Attorney, Agent, or Firm—Arthur E. Kluegel

[57]

## ABSTRACT

Disclosed is a photographic element comprising a silver halide emulsion layer having associated therewith a 3-indoloylacetanilide yellow dye-forming coupler of structure I, below:

I



wherein:

R<sub>1</sub> is an alkyl or phenyl group;

R<sub>2</sub> is a phenyl, t-butyl, cyclohexyl or naphthyl group;

X is a halogen atom or an alkoxy or alkyl group;

each R<sub>3</sub> is in the para position or either meta position relative to the anilino nitrogen and is individually selected from the group consisting of halogen atoms, and alkyl, phenyl, alkoxy, phenoxy, carbamoyl, sulfamoyl, carbonamido, sulfonamido, alkylsulfonyl, arylsulfonyl, alkoxy carbonyl, aryloxycarbonyl, acyloxy, sulfoxyl, sulfonyloxy, alkylthio, acyl and cyano groups; and n is 1, 2 or 3;

R<sub>4</sub> is a hydrogen atom or an alkyl group;

R<sub>5</sub> is a hydrogen atom or an alkyl group; and

each R<sub>6</sub> is individually a halogen atom, an alkyl group or an alkoxy group and m is 0-4;

provided that substituents may join to form a ring.

**15 Claims, No Drawings**

PHOTOGRAPHIC ELEMENT CONTAINING  
CYLACETAMIDO YELLOW DYE-FORMING  
COUPLERS

FIELD OF INVENTION

This invention relates to a photographic element comprising a support bearing at least one silver halide emulsion and at least one 3-indolylacetanilide yellow dye-forming coupler having an oxazolidine-2,4-dione coupling-off group. This invention also relates to a method for efficiently forming a stable image from said photographic element.

BACKGROUND OF INVENTION

In a silver halide color photographic element or material, a color image is formed when the element is given an imagewise exposure to light and then subjected to a color development process. In the color development process silver halide is reduced to silver as a function of exposure by a color developing agent, which is oxidized and then reacts with coupler to form dye. The spectral and stability properties of the dyes formed during photographic development are important in determining image quality and permanence. In most color photographic elements the coupler or couplers are coated in the element in the form of small dispersion droplets.

There are many references to yellow dye-forming couplers in the art. Among them are U.S. Pat. Nos. 3,973,968, 4,022,620 and 5,066,574, which disclose yellow dye-forming couplers with hydantoin-type coupling-off groups. U.S. Pat. Nos. 4,404,727 and 5,451,492 and Canadian Patent 1,039,291 disclose yellow dye-forming couplers with oxazolidinedione coupling-off groups. None of these references discloses the 3-indolylacetanilide yellow dye-forming couplers of this invention. U.S. Pat. No. 5,674,667 (EPA 751,428 A1) discloses pyrroloylacetanilide yellow dye-forming couplers with a variety of coupling-off groups. The pyrroloylacetanilide couplers of U.S. Pat. No. 5,674,667 are structurally distinct from the 3-indolylacetanilide couplers of this invention and lack the major advantages of the couplers of this invention.

The yellow dye-forming imaging and image-modifying couplers disclosed in the prior art suffer from a number of deficiencies. Generally, the dyes formed from previously disclosed yellow couplers have low extinction coefficients. This necessitates the coating of more silver and coupler, resulting in increased cost, reduced sharpness (due to additional light scattering) and less rapid processing. In addition, dyes generated from most previously disclosed yellow dye-forming couplers have insufficient thermal or dark stability, leading to undesirable losses in blue density upon long term storage of the photographic materials in which they are utilized. Furthermore, many previously disclosed yellow dye-forming couplers are of low activity, further necessitating increased coupler laydowns.

It is a problem to be solved to provide a photographic element and coupler which exhibit improved color forming ability and improved dye stability.

SUMMARY OF THE INVENTION

The invention provides a photographic element, comprising a support bearing at least one silver halide emulsion and at least one 3-indolylacetanilide yellow dye-forming coupler of structure I, below:

5

2

I



wherein:

R<sub>1</sub> is an alkyl or phenyl group;

R<sub>2</sub> is a phenyl, t-butyl, cyclohexyl or naphthyl group;

X is a halogen atom or an alkoxy or alkyl group;

each R<sub>3</sub> is in the para position or either meta position relative to the anilino nitrogen and is individually selected from the group consisting of halogen atoms, and alkyl, phenyl, alkoxy, phenoxy, carbamoyl, sulfamoyl, carbonamido, sulfonamido, alkylsulfonyl, arylsulfonyl, alkoxy carbonyl, aryloxycarbonyl, acyloxy, sulfoxyl, sulfonyloxy, alkylthio, acyl and cyano groups;

n is 1, 2 or 3;

R<sub>4</sub> is a hydrogen atom or an alkyl group;

R<sub>5</sub> is a hydrogen atom or an alkyl group; and

each R<sub>6</sub> is individually a halogen atom, an alkyl group or an alkoxy group and m is 0-4;

provided that substituents may join to form a ring.

The invention also provides a new yellow coupler and a process for forming an image in the element of the invention.

The element of the invention provides a photographic element and coupler which exhibit improved color forming ability and improved dye stability.

DETAILED DESCRIPTION OF THE INVENTION

As described, the coupler employed in the invention is represented by formula I:



wherein:

R<sub>1</sub> is an alkyl or phenyl group;

R<sub>2</sub> is a phenyl, t-butyl, cyclohexyl or naphthyl group;

X is a halogen atom or an alkoxy or alkyl group;

each R<sub>3</sub> is in the para position or either meta position relative to the anilino nitrogen and is individually selected from the group consisting of halogen atoms, and alkyl, phenyl, alkoxy, phenoxy, carbamoyl, sulfamoyl, carbonamido, sulfonamido, alkylsulfonyl, arylsulfonyl, alkoxy carbonyl, aryloxycarbonyl, acyloxy, sulfoxyl, sulfonyloxy, alkylthio, acyl and cyano groups,

arylsulfonyl, alkoxy carbonyl, aryloxycarbonyl, acyloxy, sulfoxyl, sulfonyloxy, alkylthio, acyl and cyano groups;

n is 1, 2 or 3;

R<sub>4</sub> is a hydrogen atom or an alkyl group;

R<sub>5</sub> is a hydrogen atom or an alkyl group; and

each R<sub>6</sub> is individually a halogen atom, an alkyl group or an alkoxy group and m is 0-4;

provided that substituents may join to form a ring.

In a useful embodiment R<sub>1</sub> is an alkyl group. In a preferred embodiment R<sub>2</sub> is a phenyl group. In another useful embodiment X is a halogen atom, such as chlorine or fluorine. In further useful embodiments n is 1 and R<sub>3</sub> is a carbamoyl group or a sulfamoyl group in either the 4- or 5-position relative to the NH group (X being in the 2-position). In a preferred embodiment at least one of R<sub>4</sub> or R<sub>5</sub> is an alkyl group. In another preferred embodiment both R<sub>4</sub> and R<sub>5</sub> are alkyl groups. In a particularly useful embodiment both R<sub>4</sub> and R<sub>5</sub> are methyl groups. In another particularly useful embodiment m is 0.

Preferably, one or more 3-indoloylacetanilide couplers of this invention is coated in the same layer with one or more blue-sensitive silver halide emulsions in the photographic elements of this invention. Blue-sensitive tabular grain emulsions, as described below, are particularly useful in the photographic elements of this invention.

Any alkyl groups contained in R<sub>1</sub>-R<sub>6</sub> and X may be straight chain, branched or cyclic and may be unsubstituted or substituted. The alkoxy groups comprising R<sub>6</sub> and X may be unbranched or branched and may be unsubstituted or substituted. The phenyl groups comprising R<sub>1</sub>, R<sub>2</sub> and R<sub>3</sub> may also be unsubstituted or substituted. The alkoxy carbonyl, aryloxycarbonyl, alkylthio, phenoxy, carbamoyl, sulfamoyl, carbonamido, sulfonamido, alkylsulfonyl, arylsulfonyl, acyloxy, sulfoxyl, sulfonyloxy and acyl groups comprising R<sub>3</sub> may also be substituted. Any substituent may be chosen to further substitute the R<sub>1</sub>-R<sub>6</sub> and X groups of this invention that does not adversely affect the performance of the 3-indoloylacetanilide couplers of this invention. Suitable substituents include halogen atoms, such as chlorine, alkenyl groups, alkynyl groups, aryl groups, hydroxy groups, alkoxy groups, aryloxy groups, acyl groups, acyloxy groups, alkoxy carbonyl groups, aryloxycarbonyl groups, carbonamido groups (including alkyl-, aryl-, alkoxy-, aryloxy- and alkylamino- carbonamido groups), carbamoyl groups, carbamoyloxy groups, sulfonamido groups, sulfamoyl groups, alkylthio groups, arylthio groups, sulfoxyl groups, sulfonyl groups, sulfonyloxy groups, alkoxy sulfonyl groups, aryloxysulfonyl groups, trifluoromethyl groups, cyano groups, imido groups and heterocyclic groups, such as 2-furyl, 3-furyl, 2-thienyl, 1-pyrrolyl, 2-pyrrolyl, 1-imidazolyl and N-succinimidyl groups. The phenyl groups useful for R<sub>1</sub>, R<sub>2</sub> and R<sub>3</sub> and the phenoxy groups useful for R<sub>3</sub> may suitably be substituted with one or more unbranched, branched or cyclic alkyl groups.

Useful coated levels of 3-indoloylacetanilide couplers of this invention range from about 0.05 to about 3.00 g/sq m, or more typically from 0.10 to 1.50 g/sq m.

The 3-indoloylacetanilide couplers of this invention may be utilized by dissolving them in high-boiling coupler solvents and then dispersing the organic coupler plus coupler solvent mixtures as small particles in aqueous solutions of gelatin and surfactant (via milling or homogenization).

Removable auxiliary organic solvents such as ethyl acetate or cyclohexanone may also be used in the preparation of such dispersions to facilitate the dissolution of the coupler in the organic phase. Coupler solvents useful for the practice of

this invention include aryl phosphates (e.g. trityl phosphate), alkyl phosphates (e.g. trioctyl phosphate), mixed aryl alkyl phosphates (e.g. diphenyl 2-ethylhexyl phosphate), aryl, alkyl or mixed aryl alkyl phosphonates, phosphine oxides (e.g. trioctylphosphine oxide), esters of aromatic acids (e.g. dibutyl phthalate, octyl benzoate, or benzyl salicylate) esters of aliphatic acids (e.g. acetyl tributyl citrate or dibutyl sebacate), alcohols (e.g. oleyl alcohol), phenols (e.g. p-dodecylphenol), carbonamides (e.g. N,N-dibutyldodecanamide or N-butylacetanilide), sulfoxides (e.g. bis(2-ethylhexyl)sulfoxide), sulfonamides (e.g. N,N-dibutyl-p-toluenesulfonamide) or hydrocarbons (e.g. dodecylbenzene). Additional coupler solvents and auxiliary solvents are noted in Research Disclosure, December 1989, Item 308119, p 993. Useful coupler:coupler solvent weight ratios range from about 1:0.1 to 1:8.0, with 1:0.3 to 1:2.0 being preferred. The 3-indoloylacetanilide couplers of this invention may also be dispersed and coated in latex particles or may be dispersed and coated without a high-boiling solvent or latex.

This invention provides couplers that form yellow dyes of improved color forming ability and dye stability. The improvements in dye thermal stability translate into increased image permanence on long term storage or on storage at high temperatures. The improved color forming ability enables reduced laydowns, layer thinning and the benefits associated therewith. The improved color forming ability derives from higher dye extinction coefficients (covering power) plus good coupler reactivity. This allows substantial reductions in required laydowns of yellow dye-forming couplers which can yield chemical cost reductions and layer thinning with concomitant increases in sharpness and processing rate and efficiency and to film or paper manufacturing benefits.

A further advantage of embodiments of the photographic elements of this invention is that the absorption spectra of the yellow dyes formed from the 3-indoloylacetanilide couplers of this invention are sharper cutting on the long wavelength side and produce less unwanted green light absorption and truer and more saturated yellow colors. The embodiments of this invention also provide the advantages of low density variability in response to variations in developer pH and low continued coupling when the elements are processed in a bleach solution directly after removal from developer solution. The oxazolidine coupling-off groups on the 3-indoloylacetanilide couplers of this invention, unlike other coupling-off groups such as phenoxy coupling-off groups, provide couplers with in-film pKa values sufficiently low (<10) to provide nearly full ionization in most developer solutions and thereby minimize sensitivity to variations in developer pH values. The 3-indoloylacetanilide couplers of this invention are also easily synthesized and readily dispersed. Unlike other coupling-off groups, such as hydantoins, the oxazolidinedione coupling-off groups of this invention facilitate the preparation of crystalline 3-indoloylacetanilide couplers.

Examples of oxazolidine-2,4-dione releasing 3-indoloylacetanilide couplers of this invention include, but are not limited to, A1-A24, below:

A1



A2



A3



A4



A5









13

-continued



14

A21

A22



A23



A24



The couplers of this invention may be used together with a variety of other types of couplers in the same layer or in different layers of a multilayer photographic material. Specifically contemplated is the use of the 3-indoloylacetanilide

imaging couplers of this invention in blue-sensitive photographic elements together with one or more yellow dye-forming DIR couplers, such as DIR couplers IR-1 and IR-2, below:



IR-1



IR-2

Unless otherwise specifically stated, the term substituted or substituent means any group or atom other than hydrogen bonded to the remainder of a molecule. Additionally, when the term "group" is used, it means that when a substituent group contains a substitutable hydrogen, it is also intended to encompass not only the substituent's unsubstituted form, but also its form further substituted with any substituent group or groups as herein mentioned, so long as the substituent does not destroy properties necessary for photographic utility. Suitably, a substituent group may be halogen or may be bonded to the remainder of the molecule by an atom of carbon, silicon, oxygen, nitrogen, phosphorous, or sulfur. The substituent may be, for example, halogen, such as chlorine, bromine or fluorine; nitro; hydroxyl; cyano; carboxyl; or groups which may be further substituted, such as alkyl, including straight or branched chain or cyclic alkyl, such as methyl, trifluoromethyl, ethyl, t-butyl, 3-(2,4-di-t-pentylphenoxy) propyl, and tetradecyl; alkenyl, such as ethylene, 2-butene; alkoxy, such as methoxy, ethoxy, propoxy, butoxy, 2-methoxyethoxy, sec-butoxy, hexyloxy, 2-ethylhexyloxy, tetradecyloxy, 2-(2,4-di-t-pentylphenoxy) ethoxy, and 2-dodecyloxyethoxy; aryl such as phenyl, 4-t-butylphenyl, 2,4,6-trimethylphenyl, naphthyl; aryloxy, such as phenoxy, 2-methylphenoxy, alpha- or beta-naphthoxy, and 4-tolyloxy; carbonamido, such as acetamido, benzamido, butyramido, tetradecanamido, alpha-2,4-di-t-pentyl-phenoxy)acetamido, alpha-(2,4-di-t-pentylphenoxy)butyramido, alpha-(3-pentadecylphenoxy)-hexanamido, alpha-(4-hydroxy-3-t-butylphenoxy)-tetradecanamido, 2-oxo-pyrrolidin-1-yl, 2-oxo-5-tetradecylpyrrolin-1-yl, N-methyltetradecanamido, N-succinimido, N-phthalimido, 2,5-dioxo-1-oxazolidinyl, 3-dodecyl-2,5-dioxo-1-imidazolyl, and N-acetyl-N-dodecylamino, ethoxycarbonylamino, phenoxy carbonylamino, benzoyloxycarbonylamino, hexadecyloxycarbonylamino, 2,4-di-t-butylphenoxy carbonylamino, phenylcarbonylamino, 2,5-(di-t-pentylphenyl) carbonylamino, p-dodecylphenylcarbonylamino, p-tolylcarbonylamino, N-methylureido, N,N-dimethylureido, N-methyl-N-dodecylureido, N,N-dioctadecylureido, N,N-diethyl-

N'-ethylureido, N-phenylureido, N,N-diphenylureido, N-phenyl-N-p-tolylureido, N-(m-hexadecylphenyl)ureido, N,N-(2,5-di-t-pentylphenyl)-N'-ethylureido, and t-butylcarbonamido; sulfonamido, such as 5 methylsulfonamido, benzenesulfonamido, p-tolylsulfonamido, p-dodecylbenzenesulfonamido, N-methyltetradecylsulfonamido, N,N-dipropylsulfamoylamino, and hexadecylsulfonamido; sulfamoyl, such as N-methylsulfamoyl, N-ethylsulfamoyl, 10 N,N-dipropylsulfamoyl, N-hexadecylsulfamoyl, N,N-dimethylsulfamoyl; N-[3(dodecyloxy)propyl]sulfamoyl, N-[4-(2,4-di-t-pentylphenoxy)butyl]sulfamoyl, N-methyl-N-tetradecylsulfamoyl, and N-dodecylsulfamoyl; carbamoyl, such as N-methylcarbamoyl, N,N-15 dibutylcarbamoyl, N-octadecylcarbamoyl, N-[4-(2,4-di-t-pentylphenoxy)butyl]carbamoyl, N-methyl-N-tetradecylcarbamoyl, and N,N-diethylcarbamoyl; acyl, such as acetyl, (2,4-di-t-amylphenoxy)acetyl, phenoxy carbonyl, p-dodecyloxyphenoxy carbonyl methoxycarbonyl, 20 butoxycarbonyl, tetradecyloxy carbonyl, ethoxycarbonyl, benzyloxy carbonyl, 3-pentadecyloxy carbonyl, and dodecyloxy carbonyl; sulfonyl, such as methoxysulfonyl, octyloxy sulfonyl, tetradecyloxy sulfonyl, 2-ethylhexyloxy sulfonyl, phenoxy sulfonyl, 2,4-di-t-pentylphenoxy sulfonyl, methylsulfonyl, octylsulfonyl, 2-ethylhexylsulfonyl, dodecylsulfonyl, hexadecylsulfonyl, phenylsulfonyl, 4-nonylphenylsulfonyl, and p-tolylsulfonyl; sulfonyloxy, such as dodecylsulfonyloxy, and hexadecylsulfonyloxy; sulfinyl, such as methylsulfinyl, octylsulfinyl, 2-ethylhexylsulfinyl, dodecylsulfinyl, hexadecylsulfinyl, phenylsulfinyl, 4-nonylphenylsulfinyl, and p-tolylsulfinyl; thio, such as ethylthio, octylthio, benzylthio, tetradecylthio, 2-(2,4-di-t-pentylphenoxy)ethylthio, phenylthio, 2-butoxy-5-t-octylphenylthio, and p-tolylthio; acyloxy, such as 25 acetoxy, benzyloxy, octadecanoxy, p-dodecylamido benzoyloxy, N-phenylcarbamoyloxy, N-ethylcarbamoyloxy, and cyclohexylcarbonyloxy; amine, such as phenylanilino, 2-chloroanilino, diethylamine, dodecylamine; imino, such as 1-(N-phenylimido)ethyl, 30 N-succinimido or 3-benzylhydantoinyl; phosphate, such as dimethylphosphate and ethylbutylphosphate; phosphite, such as diethyl and dihexylphosphite; a heterocyclic group, a heterocyclic oxy group or a heterocyclic thio group, each of which may be substituted and which contain a 3 to 7 membered heterocyclic ring composed of carbon atoms and at least one hetero atom selected from the group consisting of oxygen, nitrogen and sulfur, such as 2-furyl, 2-thienyl, 2-benzimidazolyl or 2-benzothiazolyl; quaternary ammonium, such as triethylammonium; and silyloxy, such as trimethylsilyloxy.

If desired, the substituents may themselves be further substituted one or more times with the described substituent groups. The particular substituents used may be selected by those skilled in the art to attain the desired photographic properties for a specific application and can include, for example, hydrophobic groups, solubilizing groups, blocking groups, releasing or releasable groups, etc. Generally, the above groups and substituents thereof may include those having up to 48 carbon atoms, typically 1 to 36 carbon atoms and usually less than 24 carbon atoms, but greater numbers are possible depending on the particular substituents selected.

The materials of the invention can be used in any of the ways and in any of the combinations known in the art. Typically, the invention materials are incorporated in a silver halide emulsion and the emulsion coated as a layer on a support to form part of a photographic element.

Alternatively, unless provided otherwise, they can be incorporated at a location adjacent to the silver halide emulsion layer where, during development, they will be in reactive association with development products such as oxidized color developing agent. Thus, as used herein, the term "associated" signifies that the compound is in the silver halide emulsion layer or in an adjacent location where, during processing, it is capable of reacting with silver halide development products.

To control the migration of various components, it may be desirable to include a high molecular weight hydrophobe or "ballast" group in coupler molecules. Representative ballast groups include substituted or unsubstituted alkyl or aryl groups containing 8 to 48 carbon atoms. Representative substituents on such groups include alkyl, aryl, alkoxy, aryloxy, alkylthio, hydroxy, halogen, alkoxy carbonyl, aryloxycarbonyl, carboxy, acyl, acyloxy, amino, anilino, carbonamido, carbamoyl, alkylsulfonyl, arylsulfonyl, sulfonamido, and sulfamoyl groups wherein the substituents typically contain 1 to 42 carbon atoms. Such substituents can also be further substituted.

The photographic elements can be single color elements or multicolor elements. Multicolor elements contain image dye-forming units sensitive to each of the three primary regions of the spectrum. Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

A typical multicolor photographic element comprises a support bearing a cyan dye image-forming unit comprised of at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler. The element can contain additional layers, such as filter layers, interlayers, overcoat layers, subbing layers, and the like.

If desired, the photographic element can be used in conjunction with an applied magnetic layer as described in *Research Disclosure*, November 1992, Item 34390 published by Kenneth Mason Publications, Ltd., Dudley Annex, 12a North Street, Emsworth, Hampshire P010 7DQ, ENGLAND, and as described in Hatsumi Kyoukai Koukai Gihou No. 94-6023, published Mar. 15, 1994, available from the Japanese Patent Office, the contents of which are incorporated herein by reference. When it is desired to employ the inventive materials in a small format film, *Research Disclosure*, June 1994, Item 36230, provides suitable embodiments.

In the following discussion of suitable materials for use in the emulsions and elements of this invention, reference will be made to *Research Disclosure*, September 1996, Item 38957, available as described above, which is referred to herein by the term "Research Disclosure". The contents of the Research Disclosure, including the patents and publications referenced therein, are incorporated herein by reference, and the Sections hereafter referred to are Sections of the Research Disclosure.

Except as provided, the silver halide emulsion containing elements employed in this invention can be either negative-

working or positive-working as indicated by the type of processing instructions (i.e. color negative, reversal, or direct positive processing) provided with the element. Suitable emulsions and their preparation as well as methods of chemical and spectral sensitization are described in Sections I through V. Various additives such as UV dyes, brighteners, antifoggants, stabilizers, light absorbing and scattering materials, and physical property modifying addenda such as hardeners, coating aids, plasticizers, lubricants and matting agents are described, for example, in Sections II and VI through VIII. Color materials are described in Sections X through XIII. Suitable methods for incorporating couplers and dyes, including dispersions in organic solvents, are described in Section X(E). Scan facilitating is described in Section XIV. Supports, exposure, development systems, and processing methods and agents are described in Sections XV to XX. The information contained in the September 1994 *Research Disclosure*, Item No. 36544 referenced above, is updated in the September 1996 *Research Disclosure*, Item No. 38957. Certain desirable photographic elements and processing steps, including those useful in conjunction with color reflective prints, are described in *Research Disclosure*, Item 37038, February 1995.

Coupling-off groups are well known in the art. Such groups can determine the chemical equivalency of a coupler, i.e., whether it is a 2-equivalent or a 4-equivalent coupler, or modify the reactivity of the coupler. Such groups can advantageously affect the layer in which the coupler is coated, or other layers in the photographic recording material, by performing, after release from the coupler, functions such as dye formation, dye hue adjustment, development acceleration or inhibition, bleach acceleration or inhibition, electron transfer facilitation, color correction and the like.

The presence of hydrogen at the coupling site provides a 4-equivalent coupler, and the presence of another coupling-off group usually provides a 2-equivalent coupler. Representative classes of such coupling-off groups include, for example, chloro, alkoxy, aryloxy, hetero-oxy, sulfonyloxy, acyloxy, acyl, heterocycl, sulfonamido, mercaptotetrazole, benzothiazole, mercaptopropionic acid, phosphonyloxy, arylthio, and arylazo. These coupling-off groups are described in the art, for example, in U.S. Pat. Nos. 2,455,169, 3,227,551, 3,432,521, 3,476,563, 3,617,291, 3,880,661, 4,052,212 and 4,134,766; and in UK. Patents and published application Nos. 1,466,728, 1,531,927, 1,533,039, 2,006, 755A and 2,017,704A, the disclosures of which are incorporated herein by reference.

Image dye-forming couplers may be included in the element such as couplers that form cyan dyes upon reaction with oxidized color developing agents which are described in such representative patents and publications as: "Farbkuppler-eine Literatur Ubersicht," published in Agfa Mitteilungen, Band III, pp. 156-175 (1961) as well as in U.S. Pat. Nos. 2,367,531; 2,423,730; 2,474,293; 2,772,162; 2,895,826; 3,002,836; 3,034,892; 3,041,236; 4,333,999; 4,746,602; 4,753,871; 4,770,988; 4,775,616; 4,818,667; 4,818,672; 4,822,729; 4,839,267; 4,840,883; 4,849,328; 4,865,961; 4,873,183; 4,883,746; 4,900,656; 4,904,575; 4,916,051; 4,921,783; 4,923,791; 4,950,585; 4,971,898; 4,990,436; 4,996,139; 5,008,180; 5,015,565; 5,011,765; 5,011,766; 5,017,467; 5,045,442; 5,051,347; 5,061,613; 5,071,737; 5,075,207; 5,091,297; 5,094,938; 5,104,783; 5,178,993; 5,813,729; 5,187,057; 5,192,651; 5,200,305; 5,202,224; 5,206,130; 5,208,141; 5,210,011; 5,215,871; 5,223,386; 5,227,287; 5,256,526; 5,258,270; 5,272,051; 5,306,610; 5,326,682; 5,366,856; 5,378,596; 5,380,638;

5,382,502; 5,384,236; 5,397,691; 5,415,990; 5,434,034; 5,441,863; EPO 0 246 616; EPO 0 250 201; EPO 0 271 323; EPO 0 295 632; EPO 0 307 927; EPO 0 333 185; EPO 0 378 898; EPO 0 389 817; EPO 0 487 111; EPO 0 488 248; EPO 0 539 034; EPO 0 545 300; EPO 0 556 700; EPO 0 556 777; EPO 0 556 858; EPO 0 569 979; EPO 0 608 133; EPO 0 636 936; EPO 0 651 286; EPO 0 690 344; German OLS 4,026,903; German OLS 3,624,777. and German OLS 3,823,049. Typically such couplers are phenols, naphthols, or pyrazoloazoles.

Couplers that form magenta dyes upon reaction with oxidized color developing agent are described in such representative patents and publications as: "Farbkuppler-eine Literature Ubersicht," published in Agfa Mitteilungen, Band III, pp. 126-156 (1961) as well as U.S. Pat. Nos. 2,311,082 and 2,369,489; 2,343,701; 2,600,788; 2,908,573; 3,062,653; 3,152,896; 3,519,429; 3,758,309; 3,935,015; 4,540,654; 4,745,052; 4,762,775; 4,791,052; 4,812,576; 4,835,094; 4,840,877; 4,845,022; 4,853,319; 4,868,099; 4,865,960; 4,871,652; 4,876,182; 4,892,805; 4,900,657; 4,910,124; 4,914,013; 4,921,968; 4,929,540; 4,933,465; 4,942,116; 4,942,117; 4,942,118; U.S. Pat. Nos. 4,959,480; 4,968,594; 4,988,614; 4,992,361; 5,002,864; 5,021,325; 5,066,575; 5,068,171; 5,071,739; 5,100,772; 5,110,942; 5,116,990; 5,118,812; 5,134,059; 5,155,016; 5,183,728; 5,234,805; 5,235,058; 5,250,400; 5,254,446; 5,262,292; 5,300,407; 5,302,496; 5,336,593; 5,350,667; 5,395,968; 5,354,826; 5,358,829; 5,368,998; 5,378,587; 5,409,808; 5,411,841; 5,418,123; 5,424,179; EPO 0 257 854; EPO 0 284 240; EPO 0 341 204; EPO 347,235; EPO 365,252; EPO 0 422 595; EPO 0 428 899; EPO 0 428 902; EPO 0 459 331; EPO 0 467 327; EPO 0 476 949; EPO 0 487 081; EPO 0 489 333; EPO 0 512 304; EPO 0 515 128; EPO 0 534 703; EPO 0 554 778; EPO 0 558 145; EPO 0 571 959; EPO 0 583 832; EPO 0 583 834; EPO 0 584 793; EPO 0 602 748; EPO 0 602 749; EPO 0 605 918; EPO 0 622 672; EPO 0 622 673; EPO 0 629 912; EPO 0 646 841; EPO 0 656 561; EPO 0 660 177; EPO 0 686 872; WO 90/10253; WO 92/09010; WO 92/10788; WO 92/12464; WO 93/01523; WO 93/02392; WO 93/02393; WO 93/07534; UK Application 2,244,053; Japanese Application 03192-350; German OLS 3,624,103; German OLS 3,912,265; and German OLS 40 08 067. Typically such couplers are pyrazolones, pyrazoloazoles, or pyrazolobenzimidazoles that form magenta dyes upon reaction with oxidized color developing agents.

Couplers that form yellow dyes upon reaction with oxidized color developing agent are described in such representative patents and publications as: "Farbkuppler-eine Literature Ubersicht," published in Agfa Mitteilungen, Band III; pp. 112-126 (1961); as well as U.S. Pat. Nos. 2,298,443; 2,407,210; 2,875,057; 3,048,194; 3,265,506; 3,447,928; 4,022,620; 4,443,536; 4,758,501; 4,791,050; 4,824,771; 4,824,773; 4,855,222; 4,978,605; 4,992,360; 4,994,361; 5,021,333; 5,053,325; 5,066,574; 5,066,576; 5,100,773; 5,118,599; 5,143,823; 5,187,055; 5,190,848; 5,213,958; 5,215,877; 5,215,878; 5,217,857; 5,219,716; 5,238,803; 5,283,166; 5,294,531; 5,306,609; 5,328,818; 5,336,591; 5,338,654; 5,358,835; 5,358,838; 5,360,713; 5,362,617; 5,382,506; 5,389,504; 5,399,474; 5,405,737; 5,411,848; 5,427,898; EPO 0 327 976; EPO 0 296 793; EPO 0 365 282; EPO 0 379 309; EPO 0 415 375; EPO 0 437 818; EPO 0 447 969; EPO 0 542 463; EPO 0 568 037; EPO 0 568 196; EPO 0 568 777; EPO 0 570 006; EPO 0 573 761; EPO 0 608 956; EPO 0 608 957; and EPO 0 628 865. Such couplers are typically open chain ketomethylene compounds.

Couplers that form colorless products upon reaction with oxidized color developing agent are described in such rep-

resentative patents as: UK. 861,138; U.S. Pat. Nos. 3,632,345; 3,928,041; 3,958,993 and 3,961,959. Typically such couplers are cyclic carbonyl containing compounds that form colorless products on reaction with an oxidized color developing agent.

Couplers that form black dyes upon reaction with oxidized color developing agent are described in such representative patents as U.S. Pat. Nos. 1,939,231; 2,181,944; 2,333,106; and 4,126,461; German OLS No. 2,644,194 and German OLS No. 2,650,764. Typically, such couplers are resorcinols or m-aminophenols that form black or neutral products on reaction with oxidized color developing agent.

In addition to the foregoing, so-called "universal" or "washout" couplers may be employed. These couplers do not contribute to image dye-formation. Thus, for example, a naphthol having an unsubstituted carbamoyl or one substituted with a low molecular weight substituent at the 2- or 3-position may be employed. Couplers of this type are described, for example, in U.S. Pat. Nos. 5,026,628, 5,151,343, and 5,234,800.

It may be useful to use a combination of couplers any of which may contain known ballasts or coupling-off groups such as those described in U.S. Pat. No. 4,301,235; U.S. Pat. No. 4,853,319 and U.S. Pat. No. 4,351,897. The coupler may contain solubilizing groups such as described in U.S. Pat. No. 4,482,629. The coupler may also be used in association with "wrong" colored couplers (e.g. to adjust levels of interlayer correction) and, in color negative applications, with masking couplers such as those described in EP 213,490; Japanese Published Application 58-172,647; U.S. Pat. Nos. 2,983,608; 4,070,191; and 4,273,861; German Applications DE 2,706,117 and DE 2,643,965; UK. Patent 1,530,272; and Japanese Application 58-113935. The masking couplers may be shifted or blocked, if desired.

Typically, couplers are incorporated in a silver halide emulsion layer in a mole ratio to silver of 0.1 to 1.0 and generally 0.1 to 0.5. Usually the couplers are dispersed in a high-boiling organic solvent in a weight ratio of solvent to coupler of 0.1 to 10.0, typically 0.1 to 2.0, although dispersions without high-boiling solvent are sometimes employed.

The invention materials may be used in association with materials that release Photographically Useful Groups (PUGS) that accelerate or otherwise modify the processing steps e.g. of bleaching or fixing to improve the quality of the image. Bleach accelerator releasing couplers such as those described in EP 193,389; EP 301,477; U.S. Pat. No. 4,163,669; U.S. Pat. No. 4,865,956; and U.S. Pat. No. 4,923,784, may be useful. Also contemplated is use of the compositions in association with nucleating agents, development accelerators or their precursors (UK Patent 2,097,140; UK. Patent 2,131,188); electron transfer agents (U.S. Pat. No. 4,859,578; U.S. Pat. No. 4,912,025); antifogging and anti color-mixing agents such as derivatives of hydroquinones, aminophenols, amines, gallic acid; catechol; ascorbic acid; hydrazides; sulfonamidophenols; and non color-forming couplers.

The invention materials may also be used in combination with filter dye layers comprising colloidal silver sol or yellow, cyan, and/or magenta filter dyes, either as oil-in-water dispersions, latex dispersions or as solid particle dispersions. Additionally, they may be used with "smearing" couplers (e.g. as described in U.S. Pat. No. 4,366,237; EP 96,570; U.S. Pat. No. 4,420,556; and U.S. Pat. No. 4,543,323.) Also, the compositions may be blocked or coated in protected form as described, for example, in Japanese Application 61/258,249 or U.S. Pat. No. 5,019,492.

The invention materials may further be used in combination with image-modifying compounds that release PUGS

such as "Developer Inhibitor-Releasing" compounds (DIR's). DIR's useful in conjunction with the compositions of the invention are known in the art and examples are described in U.S. Pat. Nos. 3,137,578; 3,148,022; 3,148,062; 3,227,554; 3,384,657; 3,379,529; 3,615,506; 3,617,291; 3,620,746; 3,701,783; 3,733,201; 4,049,455; 4,095,984; 4,126,459; 4,149,886; 4,150,228; 4,211,562; 4,248,962; 4,259,437; 4,362,878; 4,409,323; 4,477,563; 4,782,012; 4,962,018; 4,500,634; 4,579,816; 4,607,004; 4,618,571; 4,678,739; 4,746,600; 4,746,601; 4,791,049; 4,857,447; 4,865,959; 4,880,342; 4,886,736; 4,937,179; 4,946,767; 4,948,716; 4,952,485; 4,956,269; 4,959,299; 4,966,835; 4,985,336 as well as in patent publications GB 1,560,240; GB 2,007,662; GB 2,032,914; GB 2,099,167; DE 2,842,063, DE 2,937,127; DE 3,636,824; DE 3,644,416 as well as the following European Patent Publications: 272,573; 335,319; 336,411; 346,899; 362,870; 365,252; 365,346; 373,382; 376,212; 377,463; 378,236; 384,670; 396,486; 401,612; 401,613.

Such compounds are also disclosed in "Developer-Inhibitor-Releasing (DIR) Couplers for Color Photography," C. R. Barr, J. R. Thirtle and P. W. Vittum in *Photographic Science and Engineering*, Vol. 13, p. 174 (1969), incorporated herein by reference. Generally, the developer inhibitor-releasing (DIR) couplers include a coupler moiety and an inhibitor coupling-off moiety (IN). The inhibitor-releasing couplers may be of the time-delayed type (DIAR couplers) which also include a timing moiety or chemical switch which produces a delayed release of inhibitor. Examples of typical inhibitor moieties are: oxazoles, thiazoles, diazoles, triazoles, oxadiazoles, thiadiazoles, oxathiazoles, thiatriazoles, benzotriazoles, tetrazoles, benzimidazoles, indazoles, isoindazoles, mercaptotetrazoles, selenotetrazoles, mercaptobenzothiazoles, selenobenzothiazoles, mercaptobenzoxazoles, selenobenzoxazoles, mercaptobenzimidazoles, selenobenzimidazoles, benzodiazoles, mercaptooxazoles, mercaptothiadiazoles, mercaptothiazoles, mercaptotriazoles, mercaptooxadiazoles, mercaptodiazoles, mercaptoxathiazoles, telleurotetrazoles or benzisodiazoles. In a preferred embodiment, the inhibitor moiety or group is selected from the following formulas:



wherein  $R_1$  is selected from the group consisting of straight and branched alkyls of from 1 to about 8 carbon atoms, benzyl, phenyl, and alkoxy groups and such groups containing none, one or more than one such substituent;  $R_2$  is selected from  $R_1$  and  $-SR_2$ ;  $R_3$  is a straight or branched alkyl group of from 1 to about 5 carbon atoms and  $p$  is from

1 to 3; and  $R_{IV}$  is selected from the group consisting of hydrogen, halogens and alkoxy, phenyl and carbonamido groups,  $-COOR_V$  and  $-NHCOOR_V$  wherein  $R_V$  is selected from substituted and unsubstituted alkyl and aryl groups.

Although it is typical that the coupler moiety included in the developer inhibitor-releasing coupler forms an image dye corresponding to the layer in which it is located, it may also form a different color as one associated with a different film layer. It may also be useful that the coupler moiety included in the developer inhibitor-releasing coupler forms colorless products and/or products that wash out of the photographic material during processing (so-called "universal" couplers).

A compound such as a coupler may release a PUG directly upon reaction of the compound during processing, or indirectly through a timing or linking group. A timing group produces the time-delayed release of the PUG such groups using an intramolecular nucleophilic substitution reaction (U.S. Pat. No. 4,248,962); groups utilizing an electron transfer reaction along a conjugated system (U.S. Pat. Nos. 4,409,323; 4,421,845; 4,861,701, Japanese Applications 57-188035; 58-98728; 58-209736; 58-209738); groups that function as a coupler or reducing agent after the coupler reaction (U.S. Pat. No. 4,438,193; U.S. Pat. No. 4,618,571) and groups that combine the features described above. It is typical that the timing group is of one of the formulas:



wherein IN is the inhibitor moiety, Z is selected from the group consisting of nitro, cyano, alkylsulfonyl; sulfamoyl ( $-SO_2NR_2$ ); and sulfonamido ( $-NRSO_2R$ ) groups; q is 0 or 1; and  $R_{VI}$  is selected from the group consisting of substituted and unsubstituted alkyl and phenyl groups. The oxygen atom of each timing group is bonded to the coupling-off position of the respective coupler moiety of the DIAR.

The timing or linking groups may also function by electron transfer down an unconjugated chain. Linking groups are known in the art under various names. Often they have been referred to as groups capable of utilizing a hemiacetal or iminoketal cleavage reaction or as groups capable of utilizing a cleavage reaction due to ester hydrolysis such as U.S. Pat. No. 4,546,073. This electron transfer down an unconjugated chain typically results in a relatively fast decomposition and the production of carbon dioxide, formaldehyde, or other low molecular weight by-products. The groups are exemplified in EP 464,612, EP 523,451, U.S. Pat. No. 4,146,396, Japanese Kokai 60-249148 and 60-249149.

Suitable developer inhibitor-releasing couplers for use in the present invention include, but are not limited to, the following:



D1

5  
1015  
20  
25  
3035  
4045  
50  
5560  
65

-continued

D5



D7

D8



**25**

-continued



D9



D10



D11

**26**

-continued



D12

It is also contemplated that the concepts of the present invention may be employed to obtain reflection color prints as described in *Research Disclosure*, November 1979, Item 18716, available from Kenneth Mason Publications, Ltd, Dudley Annex, 12a North Street, Emsworth, Hampshire PO101 7DQ, England, incorporated herein by reference. Materials of the invention may be coated on pH adjusted support as described in U.S. Pat. No. 4,917,994; on a support with reduced oxygen permeability (EP 553,339); with epoxy solvents (EP 164,961); with nickel complex stabilizers (U.S. Pat. No. 4,346,165; U.S. Pat. No. 4,540,653 and U.S. Pat. No. 4,906,559 for example); with ballasted chelating agents such as those in U.S. Pat. No. 4,994,359 to reduce sensitivity to polyvalent cations such as calcium; and with stain reducing compounds such as described in U.S. Pat. No. 5,068,171. Other compounds useful in combination with the invention are disclosed in Japanese Published Applications described in Derwent Abstracts having accession numbers as follows: 90-072,629; 90-072,630; 90-072,631; 90-072,632; 90-072,633; 90-072,634; 90-077,822; 90-078,229; 90-078,230; 90-079,336; 90-079,337; 90-079,338; 90-079,690; 90-079,691; 90-080,487; 90-080,488; 90-080,489; 90-080,490; 90-080,491; 90-080,492; 90-080,494; 90-085,928; 90-086,669; 90-086,670; 90-087,360; 90-087,361; 90-087,362; 90-087,363; 90-087,364; 90-088,097; 90-093,662; 90-093,663; 90-093,664; 90-093,665; 90-093,666; 90-093,668; 90-094,055; 90-094,056; 90-103,409; 83-62,586; 83-09,959.

Conventional radiation-sensitive silver halide emulsions can be employed in the practice of this invention. Such emulsions are illustrated by *Research Disclosure*, Item 38755, September 1996, I. Emulsion grains and their preparation.

Especially useful in this invention are tabular grain silver halide emulsions. Tabular grains are those having two par-

55

60

65

allel major crystal faces and having an aspect ratio of at least 2. The term "aspect ratio" is the ratio of the equivalent circular diameter (ECD) of a grain major face divided by its thickness (t). Tabular grain emulsions are those in which the tabular grains account for at least 50 percent (preferably at least 70 percent and optimally at least 90 percent) of total grain projected area. Preferred tabular grain emulsions are those in which the average thickness of the tabular grains is less than 0.3 micrometer (preferably thin—that is, less than 0.2 micrometer and most preferably ultrathin—that is, less than 0.07 micrometer). The major faces of the tabular grains can lie in either {111} or {100} crystal planes. The mean ECD of tabular grain emulsions rarely exceeds 10 micrometers and more typically is less than 5 micrometers.

In their most widely used form tabular grain emulsions are high bromide {111} tabular grain emulsions. Such emulsions are illustrated by Kofron et al U.S. Pat. No. 4,439,520, Wilgus et al U.S. Pat. No. 4,434,226, Solberg et al U.S. Pat. No. 4,433,048, Maskasky U.S. Pat. Nos. 4,435,501, 4,463,087 and 4,173,320, Daubendiek et al U.S. Pat. Nos. 4,414,310 and 4,914,014, Sowinski et al U.S. Pat. No. 4,656,122, Pigglin et al U.S. Pat. Nos. 5,061,616 and 5,061,609, Tsaur et al U.S. Pat. Nos. 5,147,771, '772, '773, 5,171,659 and U.S. Pat. No. 5,252,453, Black et al U.S. Pat. Nos. 5,219,720 and 5,334,495, Delton U.S. Pat. Nos. 5,310,644, 5,372,927 and 5,460,934, Wen U.S. Pat. No. 5,470,698, Fenton et al U.S. Pat. No. 5,476,760, Eshelman et al U.S. Pat. Nos. 5,612,175 and 5,614,359, and Irving et al U.S. Pat. No. 5,667,954.

Ultrathin high bromide {111} tabular grain emulsions are illustrated by Daubendiek et al U.S. Pat. Nos. 4,672,027, 4,693,964, 5,494,789, 5,503,971 and 5,576,168, Antoniades et al U.S. Pat. No. 5,250,403, Olm et al U.S. Pat. No. 5,503,970, Deaton et al U.S. Pat. No. 5,582,965, and Maskasky U.S. Pat. No. 5,667,955.

High bromide {100} tabular grain emulsions are illustrated by Mignot U.S. Pat. Nos. 4,386,156 and 5,386,156.

High chloride {111} tabular grain emulsions are illustrated by Wey U.S. Pat. No. 4,399,215, Wey et al U.S. Pat. No. 4,414,306, Maskasky U.S. Pat. Nos. 4,400,463, 4,713,323, 5,061,617, 5,178,997, 5,183,732, 5,185,239, 5,399,478 and 5,411,852, and Maskasky et al U.S. Pat. Nos. 5,176,992 and 5,178,998. Ultrathin high chloride {111} tabular grain emulsions are illustrated by Maskasky U.S. Pat. Nos. 5,271,858 and 5,389,509.

High chloride {100} tabular grain emulsions are illustrated by Maskasky U.S. Pat. Nos. 5,264,337, 5,292,632, 5,275,930 and 5,399,477, House et al U.S. Pat. No. 5,320,938, Brust et al U.S. Pat. No. 5,314,798, Szajewski et al U.S. Pat. No. 5,356,764, Chang et al U.S. Pat. Nos. 5,413,904 and 5,663,041, Oyamada U.S. Pat. No. 5,593,821, Yamashita et al U.S. Pat. Nos. 5,641,620 and 5,652,088, Saitou et al U.S. Pat. No. 5,652,089, and Oyamada et al U.S. Pat. No. 5,665,530. Ultrathin high chloride {100} tabular grain emulsions can be prepared by nucleation in the presence of iodide, following the teaching of House et al and Chang et al, cited above.

The emulsions can be surface-sensitive emulsions, i.e., emulsions that form latent images primarily on the surfaces of the silver halide grains, or the emulsions can form internal latent images predominantly in the interior of the silver halide grains. The emulsions can be negative-working emulsions, such as surface-sensitive emulsions or unfogged internal latent image-forming emulsions, or direct-positive emulsions of the unfogged, internal latent image-forming type, which are positive-working when development is

conducted with uniform light exposure or in the presence of a nucleating agent. Tabular grain emulsions of the latter type are illustrated by Evans et al U.S. Pat. No. 4,504,570.

Photographic elements can be exposed to actinic radiation, typically in the visible region of the spectrum, to form a latent image and can then be processed to form a visible dye image. Processing to form a visible dye image includes the step of contacting the element with a color developing agent to reduce developable silver halide and oxidize the color developing agent. Oxidized color developing agent in turn reacts with the coupler to yield a dye. If desired "Redox Amplification" as described in Research Disclosure XVIIIB(5) may be used.

With negative-working silver halide, the processing step described above provides a negative image. One type of such element, referred to as a color negative film, is designed for image capture. Speed (the sensitivity of the element to low light conditions) is usually critical to obtaining sufficient image in such elements. Such elements are typically silver bromoiodide emulsions coated on a transparent support and may be processed, for example, in known color negative processes such as the Kodak C-41 process as described in The British Journal of Photography Annual of 1988, pages 191-198. If a color negative film element is to be subsequently employed to generate a viewable projection print as for a motion picture, a process such as the Kodak ECN-2 process described in the H-24 Manual available from Eastman Kodak Co. may be employed to provide the color negative image on a transparent support. Color negative development times are typically 3' 15" or less and desirably 90 or even 60 seconds or less.

The photographic element of the invention can be incorporated into exposure structures intended for repeated use or exposure structures intended for limited use, variously referred to by names such as "single use cameras", "lens with film", or "photosensitive material package units".

Another type of color negative element is a color print. Such an element is designed to receive an image optically printed from an image capture color negative element. A color print element may be provided on a reflective support for reflective viewing (e.g. a snap shot) or on a transparent support for projection viewing as in a motion picture. Elements destined for color reflection prints are provided on a reflective support, typically paper, employ silver chloride emulsions, and may be optically printed using the so-called negative-positive process where the element is exposed to light through a color negative film which has been processed as described above. The element is sold with instructions to process using a color negative optical printing process, for example the Kodak RA-4 process, as generally described in PCT WO 87/04534 or U.S. Pat. No. 4,975,357, to form a positive image. Color projection prints may be processed, for example, in accordance with the Kodak ECP-2 process as described in the H-24 Manual. Color print development times are typically 90 seconds or less and desirably 45 or even 30 seconds or less.

A reversal element is capable of forming a positive image without optical printing. To provide a positive (or reversal) image, the color development step is preceded by development with a non-chromogenic developing agent to develop exposed silver halide, but not form dye, and followed by uniformly fogging the element to render unexposed silver halide developable. Such reversal emulsions are typically sold with instructions to process using a color reversal process such as the Kodak E-6 process as described in The British Journal of Photography Annual of 1988, page 194. Alternatively, a direct positive emulsion can be employed to obtain a positive image.

**29**

The above elements are typically sold with instructions to process using the appropriate method such as the mentioned color negative (Kodak C-41), color print (Kodak RA-4), or reversal (Kodak E-6) process.

Preferred color developing agents are p-phenylenediamines such as:

4-amino-N,N-diethylaniline hydrochloride,  
4-amino-3-methyl-N,N-diethylaniline hydrochloride,

**30**

4-amino-3-methyl-N-ethyl-N-(2-methanesulfonamidoethyl)aniline sesquisulfate hydrate,  
4-amino-3-methyl-N-ethyl-N-(2-hydroxyethyl)aniline sulfate,

4-amino-3-(2-methanesulfonamidoethyl)-N,N-diethylaniline hydrochloride, and  
4-amino-N-ethyl-N-(2-methoxyethyl)-m-toluidine di-p-toluene sulfonic acid.

Development is usually followed by the conventional steps of bleaching, fixing, or bleach-fixing, to remove silver or silver halide, washing, and drying.



-continued



## Synthesis Example

## Synthesis of 2

Dimethylacetamide (700 mL) was placed in a 2 liter 3-neck round bottom flask equipped with a thermometer, mechanical stirrer and addition funnel. The mechanically stirred liquid was cooled to -5° C. with an ice/acetone bath. Phosphorous oxychloride (POCl<sub>3</sub>, 100 mL, 1.07 moles) was added dropwise over a sixty minute period. During this time the temperature rose to 5° C. After addition was complete, 2-phenyl indole 1 (193 grams, 1.0 mole) was added portionwise over a 10 minute period. The ice bath was removed and replaced with a heating mantle. The temperature was raised to ~50° C. for one hour and then to ~85° C. for two hours. Thin layer chromatography (TLC, ethyl acetate 20%, heptane 80%) on the solution showed no starting material and only faint impurities. The solution was poured into a 3 liter mixture of crushed ice and water with stirring. Within a few minutes the stirred suspension set up to a dark green solid. To this, 500 grams of 50% aqueous sodium hydroxide was added. The mixture exothermed from 10° C. to 50° C. The suspension broke up and became orange colored. The mechanically stirred suspension was heated to 95° C. for one hour, then cooled to 50° C., and 250 mL of concentrated HCl was added slowly. The mixture was mechanically stirred overnight. The solid which formed was filtered, and recrystallized from methanol to give a tan solid 2 (207 grams, 88% yield). The structure was confirmed by NMR spectroscopy.

## Synthesis of 3

The indole 2 (57 grams, 0.24 moles) was placed in a 3 liter Morton flask, equipped with a mechanical stirrer and thermometer. The flask was charged with 450 mL of toluene and the suspension was vigorously stirred. To this, diethylsulfate (38 mL, 0.29 moles) was added, then 50% aqueous sodium hydroxide (38 mL, 0.72 moles) was added, followed by a catalytic amount of tetrabutylammonium bromide (1 gram). After fifteen minutes an exotherm was noticed. Within an two hours the solid was in solution. TLC (ethyl acetate 20%, heptane 80%) showed no starting material 2, and one new spot. The solution was diluted with two liters of water and one liter of ethyl acetate. The aqueous layer was separated from the organic layer and discarded. The organic layer was dried with magnesium sulfate, filtered and concentrated to near dryness. To this, 0.3 liters of low-boiling ligroin was added. The slightly colored solid which formed was filtered and air dried to give 58.1 grams of 3 (92%). The structure was confirmed by NMR spectroscopy.

## Synthesis of 4

A mechanically stirred solution of 3 in dimethylformamide (150 mL) and dimethylcarbonate (185 mL, 2.2 moles) was treated in portions with potassium tert-butoxide (74 grams, 0.66 moles). The solution was stirred at ambient temperatures for two hours. TLC (ethyl acetate 25%, heptane 75%) showed no starting material and one new spot.



15 One liter of cold dilute HCl was added slowly to the reaction mixture. The solid that formed was filtered and air dried to give 68 grams of a yellow solid 4 (96% yield). The structure was confirmed by NMR spectroscopy.

## Synthesis of 6

20 A stirred suspension of 4 (13.2 grams, 0.04 moles) and benzamide, 4-amino-3-chloro-N-octyl 5(11.6 grams, 0.04 moles) in 500 mL of xylenes was heated to reflux into a Dean Stark trap for eight hours. During this time, 400 mL of xylenes was removed via the Dean Stark trap. After four 25 hours, TLC (ethyl acetate 40%, heptane 60%) showed no starting material and one major new spot. The solution was cooled to room temperature and stirred for 24 hours. During this time period a solid crystallized from the solution. The mixture was diluted with one liter of heptane. The solid was filtered, washed twice with low boiling ligroin and air dried to give 21.6 grams (92% yield) of a tan solid. The structure was confirmed by NMR and mass spectroscopy.

## Synthesis of 7

25 Stirred suspension of 6 (21.6 grams, 0.038 moles) in 150 mL of toluene was heated to 80° C. until everything was in solution. Dibromodimethylhydantoin (6.5 grams, 0.023 moles) was added to the solution in one portion. The reaction mixture was stirred at 80° C. for one hour. TLC (ethyl acetate 40%, heptane 60%) showed no starting material and one major new spot. The reaction mixture was cooled to room temperature, placed on a column of silica gel and chromatographed, eluting with heptane 90%, ethyl acetate 10% up to heptane 70%, ethyl acetate 30%. The solvent was removed under reduced pressure to give 7 as a red oil (18.7 30 grams, 98%). The structure was confirmed by NMR spectroscopy.

## Synthesis of A5

35 A solution of 2,4-oxazolidinedione, 5,5-dimethyl 8 (6.2 grams, 0.048 moles) in 50 mL of dimethylacetamide (DMAc) was treated with potassium tert-butoxide (4.0 grams, 0.036 moles) in one portion. The solution was stirred at ambient temperature for ten minutes. To this, a solution of 7 (15.6 grams, 0.024 moles) in 100 mL of DMAc was added in one portion. The reaction mixture was stirred at ambient 40 temperature for thirty minutes. TLC (ethyl acetate 40%, heptane 60%) showed no starting material and one major new spot. The reaction was partitioned between dilute HCl and ethyl acetate. The product was extracted into the organic layer, dried with magnesium sulfate, and concentrated to an 50 oil. The oil was dissolved in toluene and chromatographed, eluting with heptane 5%, ethyl acetate 95% up to heptane 65%, ethyl acetate 35%. The solvent was removed under reduced pressure to give a yellow oil. The oil was dissolved in 1-chlorobutane and diluted with heptane until the solution was cloudy. The mixture was stirred at ambient temperatures 55 for 24 hours. During this time period a solid crystallized from the mixture. The solid was filtered and air dried to give 60 oil.

8.5 grams (51% yield) of A5. The structure was confirmed by NMR and mass spectroscopy. Combustion analysis, theory: C 67.0, H 6.2, N 8.0, Cl 5.1, Found: C 66.9, H 6.2, N 8.0, Cl 5.5.

#### Photographic Examples

##### EXAMPLE 1

###### Illustration of the Superior Color-Forming Ability and Thermal Dye Stability Provided by 3-Indoloylacetanilide Couplers and Photographic Elements of this Invention.

Because of the high activity of the oxazolidine-2,4-dione-releasing 3-indoloylacetanilide couplers of this invention and because of the high extinction coefficients of the yellow dyes that they form, they have superior color-forming ability. Furthermore, the dyes formed from the couplers of this invention have superior stability toward long term storage or storage at elevated temperatures. Both of these advantages are illustrated in this comparative example.

For this example, comparative coupler C1 and couplers A1 and A2 of this invention were each dispersed and coated with the high-boiling coupler solvent tritolyl phosphate (S-1, mixed isomers). The dispersions were prepared by adding an oil phase containing a 1:0.5:3 weight ratio of coupler:S-1:ethyl acetate to an aqueous phase containing gelatin and the dispersing agent ALKANOL XC (DuPont) (mixed isomers of triisopropyl-2-naphthalene sulfonic acid, sodium salt) in a 10:1 weight ratio. The mixture was then passed through a colloid mill to disperse the oil phase in the aqueous phase as small particles. On coating, the ethyl acetate auxiliary solvent evaporates. The coupler dispersions, consisting of approximately 4% coupler and 6% gelatin, were coated together with a silver iodobromide (3.5% iodide) emulsion on a transparent support. The coating structure is shown in Table I with laydowns in g/sq m given in parentheses. The structure of comparative couplers C1 is provided after Table I.

Comparative coupler C1 is widely used in commercial color photographic materials, including color negative films and color paper. To provide suitable dye densities and compensate for its lower activity and dye covering power, comparative coupler C1 was coated at a higher laydown of 1.51 mmole/sq m. The high activities and high dye extinction coefficients of couplers A1 and A2 of this invention permitted coating them at a lower laydown of 1.08 mmole/sq m, providing a significant advantage.

TABLE I

|                                                                     |                                            |
|---------------------------------------------------------------------|--------------------------------------------|
| Overcoat:                                                           | Gelatin (2.69)                             |
|                                                                     | Bis(vinylsulfonyl)methane Hardener (0.129) |
| A Comparative Coupler C1 @ 1.51 mmole/sq m (0.978) & S-1 (0.489)    |                                            |
| or B Comparative Coupler A1 @ 1.08 mmole/sq m (0.797) & S-1 (0.398) |                                            |
| or C Comparative Coupler A2 @ 1.08 mmole/sq m (0.812) & S-1 (0.406) |                                            |
| 0.7 $\mu$ m Silver Iodobromide Emulsion (0.755 Ag)                  |                                            |
| Gelatin (3.77)                                                      |                                            |
| Cellulose Acetate Butyrate Support                                  |                                            |

TABLE I-continued



1:1:3 weight ratio of coupler:S-2:ethyl acetate to an aqueous phase containing gelatin and the dispersing agent ALKANOL XC (DuPont) in a 10:1 weight ratio. The mixture was then passed through a colloid mill to disperse the oil phase in the aqueous phase as small particles. The dispersions contained about 4% by weight of coupler and 6% by weight of gelatin. On coating the ethyl acetate auxiliary solvent evaporates. The coupler dispersions were coated together with a silver iodobromide (3.5% iodide) emulsion on a transparent support. The coating structure is shown in Table IV with laydowns in g/sq m given in parentheses. In this example, all couplers were coated at the same laydown of 1.08 mmole/sq m.

TABLE IV

|                                                                   |
|-------------------------------------------------------------------|
| Overcoat: Gelatin (2.69)                                          |
| Bis(vinylsulfonyl)methane Hardener(0.129)                         |
| D Comparative Coupler C1 @ 1.08 mmole/sq m (0.698) & S-2 (0.698)  |
| or E Invention Coupler A1 @ 1.08 mmole/sq m (0.797) & S-2 (0.797) |
| or F Invention Coupler A3 @ 1.08 mmole/sq m (0.836) & S-2 (0.836) |
| or G Invention Coupler A4 @ 1.08 mmole/sq m (0.776) & S-2 (0.776) |
| 0.7 $\mu$ m Silver Iodobromide Emulsion (0.755 Ag)                |
| Gelatin (3.77)                                                    |
| Cellulose Acetate Butyrate Support                                |

Samples of the hardened films in Table IV were exposed and processed as in Example 1. Status M blue gamma values were determined as in Example 1 and are given in Table V. Blue densities were also measured for exposed and processed film samples both immediately after processing and after storage at 80C/50% RH as in Example 1, and the values of % fade/wk obtained from these measurements are reported in Table V. Epsilon (extinction coefficient) values for the dyes generated in the films were also determined and are also reported in Table V. From the comparative data in

Table V it can be seen that the couplers of this invention, A1, A3 and A4, give higher gamma values and dyes with better thermal stability and higher epsilon values than comparative coupler C1. The features of the couplers of this invention illustrated in Table V are both unexpected and highly desirable.

TABLE V

| Coating | Coupler          | Blue Gamma | % Fade/week @ 80 C/50% RH | Epsilon sq cm/mmole |
|---------|------------------|------------|---------------------------|---------------------|
| D       | C1 (Comparative) | 1.24       | 3.2                       | 17,500              |
| E       | A1 (Invention)   | 1.54       | 1.0                       | 22,000              |
| F       | A3 (Invention)   | 1.53       | 0.3                       | 26,500              |
| G       | A4 (Invention)   | 1.44       | 0.1                       | 26,500              |

15

## EXAMPLE 3

## Multilayer Film Structure Comprising a Yellow Coupler of This Invention

The multilayer film structure utilized for this example is shown schematically in Table VI. Structures of components not provided previously are given immediately following Table VI. Component laydowns are provided in units of g/sq m unless otherwise indicated. This composition may also be coated on a support, such as polyethylene naphthalate, containing a magnetic recording layer. The use of the 3-indoloylacetanilide imaging coupler A5 of this invention provides reduced coupler laydowns, layer thinning and improved sharpness. The color negative film described in Table VI may be processed using KODAK FLEXICOLOR C-41 chemistry to yield excellent latitude, sharpness, color and interlayer interimage.

TABLE VI

## MULTILAYER FILM STRUCTURE

|                        |                                                                                                                                                                                                                                                                                                                                                                                                                                                                                                                                                                                                                                                                                                                                                                                                                                                                                                                                                                                                                                                                                                                                                                                                                                                                                                            |
|------------------------|------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| 1 Overcoat & UV Layer: | Matte Beads<br>UV Absorbers UV-1 (0.108), UV-2 (0.108) & S-1 (0.151)<br>Silver Bromide Lippmann Emulsion (0.215 Ag)<br>Gelatin (1.237)<br>Bis(vinylsulfonyl)methane Hardener (1.75% of Total Gelatin)<br>A5 (0.190) (Invention Image Coupler) & S-1 (0.190)<br>IR-1 (0.076) DIR Coupler & S-1 (0.038)<br>B-1 (0.0054) BARC & S-3 (0.0070)<br>Blue Sensitive Silver Iodobromide Emulsion (0.339 Ag),<br>4.1 mole % Iodide T-Grain (2.9 $\times$ 0.12 $\mu$ m)<br>Blue Sensitive Silver Iodobromide Emulsion (0.097 Ag)<br>4.1 mole % Iodide T-Grain (1.9 $\times$ 0.14 $\mu$ m)<br>Gelatin (0.726)<br>A5 (0.870) (Invention) & S-1 (0.870)<br>IR-1 (0.076) (Invention DIR Coupler) & S-1 (0.038)<br>B-1 (0.022) & S-3 (0.0028)<br>CC-1 (0.032) & S-2 (0.064)<br>IR-4 (0.032) & S-2 (0.064)<br>Blue Sensitive Silver Iodobromide Emulsion (0.358 Ag),<br>4.1 mole % Iodide T-Grain (1.9 $\times$ 0.14 $\mu$ m)<br>Blue Sensitive Silver Iodobromide Emulsion (0.242 Ag),<br>1.3 mole % Iodide T-Grain (0.54 $\times$ 0.08 $\mu$ m)<br>Blue Sensitive Silver Iodobromide Emulsion (0.222 Ag)<br>1.5 mole % Iodide T-Grain (0.77 $\times$ 0.14 $\mu$ m)<br>Gelatin (1.685)<br>R-1 (0.086) & S-2 (0.139) & ST-2 (0.012)<br>YD-2 Filter Dye (0.054)<br>Gelatin (0.646)<br>M-1(0.072) Magenta Dye-Forming Coupler |
| 2 Fast Yellow H Layer: |                                                                                                                                                                                                                                                                                                                                                                                                                                                                                                                                                                                                                                                                                                                                                                                                                                                                                                                                                                                                                                                                                                                                                                                                                                                                                                            |
| 3 Slow Yellow Layer:   |                                                                                                                                                                                                                                                                                                                                                                                                                                                                                                                                                                                                                                                                                                                                                                                                                                                                                                                                                                                                                                                                                                                                                                                                                                                                                                            |
| 4 Yellow Filter Layer: |                                                                                                                                                                                                                                                                                                                                                                                                                                                                                                                                                                                                                                                                                                                                                                                                                                                                                                                                                                                                                                                                                                                                                                                                                                                                                                            |
| 5 Fast Magenta         |                                                                                                                                                                                                                                                                                                                                                                                                                                                                                                                                                                                                                                                                                                                                                                                                                                                                                                                                                                                                                                                                                                                                                                                                                                                                                                            |

20

25

30

TABLE VI-continued

| MULTILAYER FILM STRUCTURE    |                                                                                                                                                                                                                                                                                                                                                                                |
|------------------------------|--------------------------------------------------------------------------------------------------------------------------------------------------------------------------------------------------------------------------------------------------------------------------------------------------------------------------------------------------------------------------------|
| Layer:                       | & S-1 (0.065)<br>& ST-1 (0.0072), Addendum, R-2 (0.009)<br>MM-1 (0.052) Masking Coupler & S-1 (0.104)<br>IR-3 (.030) DIR Coupler & S-2 (0.060)<br>B-1 (0.003) & S-3 (0.004)<br>Green Sensitive Silver Iodobromide<br>Emulsion (0.465 Ag),<br>4.0 mole % Iodide T-Grain (1.60 x 0.12 $\mu$ m)<br>Gelatin (0.973)                                                                |
| 6 Mid Magenta                | M-1 (0.119) & S-1 (0.107) & ST-1 (0.012)<br>MM-1 (0.113) & S-1 (0.226), R-2 (0.015)<br>IR-2 (0.043) DIR Coupler & S-2 (0.043)<br>Green Sensitive Silver Iodobromide<br>Emulsion (0.237 Ag),<br>4.0 mole % Iodide T-Grain (1.20 x 0.11 $\mu$ m)<br>Green Sensitive Silver Iodobromide Emulsion (0.237 Ag)<br>4.0 mole % Iodide T-Grain (1.00 x 0.12 $\mu$ m)<br>Gelatin (1.167) |
| 7 Slow Magenta               | M-1 (0.258) & S-1 (0.232) & ST-1 (0.026)<br>MM-1 (0.082) & S-1 (0.164)<br>IR-2 (0.011) & S-2(0.011)<br>Green Sensitive Silver Iodobromide<br>Emulsion (0.330 Ag),<br>3.5 mole % Iodide T-Grain (0.90 x 0.12 $\mu$ m)<br>Green Sensitive Silver Iodobromide<br>Emulsion (0.124 Ag),<br>1.5 mole % Iodide T-Grain (0.50 x 0.08 $\mu$ m)<br>Gelatin (1.033)                       |
| 8 Interlayer:                | R-1 (0.086) Interlayer Scavenger, S-2 (0.139)<br>& ST-2 (0.012)<br>Gelatin (0.538)                                                                                                                                                                                                                                                                                             |
| 9 Fast Cyan                  | CC-1 (0.176) Cyan Dye-Forming Coupler & S-2 (0.203)<br>CM-1 (0.022) Masking Coupler<br>IR-4 (0.027) DIAR Coupler & S-2 (0.054)<br>Red Sensitive Silver Iodobromide Emulsion (0.568 Ag),<br>4.1 mole % Iodide T-Grain (1.7 x 0.12 $\mu$ m)<br>Gelatin (0.878)                                                                                                                   |
| 10 Mid Cyan                  | CC-1 (0.163) & S-2 (0.182)<br>CM-1 (0.032)<br>B-1 (0.008) & S-3 (0.010)<br>IR-4 (0.019) & S-2 (0.038)<br>Red Sensitive Silver Iodobromide Emulsion (0.186 Ag),<br>4.1 mole % Iodide T-Grain (1.2 x 0.11 $\mu$ m)<br>Red Sensitive Silver Iodobromide Emulsion (0.228 Ag),<br>4.1 mole % Iodide T-Grain (0.91 x 0.11 $\mu$ m)<br>Gelatin (1.033)                                |
| 11 Slow Cyan                 | CC-1 (0.511) & S-2 (0.542)<br>IR-4 (0.026) & S-2 (0.052)<br>CM-1 (0.031)<br>B-1 (0.056) & S-3 (0.073)<br>Red Sensitive Silver Iodobromide Emulsion (0.444 Ag),<br>1.5 mole % Iodide T-Grain (0.54 x 0.06 $\mu$ m)<br>Red Sensitive Silver Iodobromide Emulsion (0.289 Ag)<br>4.1 mole % Iodide T-Grain (0.53 x 0.12 $\mu$ m)<br>Gelatin (1.612)                                |
| 12 Antihalation              | Gray Silver (0.135)<br>UV-1 (0.075), UV-2 (0.030), S-1 (0.042) S-4 (0.015)<br>YD-1 (0.034), MD-1 (0.018) & S-5 (0.018)<br>CD-1 (0.025) & S-2 (0.125)<br>R-1 (0.161), S-2 (0.261) & ST-2 (0.022)<br>Gelatin (2.04)                                                                                                                                                              |
| Cellulose Triacetate Support |                                                                                                                                                                                                                                                                                                                                                                                |



TABLE VI-continued

## MULTILAYER FILM STRUCTURE



TABLE VI-continued



TABLE VI-continued

| MULTILAYER FILM STRUCTURE |                      |
|---------------------------|----------------------|
|                           | MD-1                 |
|                           | MM-1                 |
|                           | R-1                  |
|                           | R-2                  |
|                           | S-1<br>mixed isomers |
|                           | S-2                  |

TABLE VI-continued

## MULTILAYER FILM STRUCTURE



S-3



S-4



S-5



ST-1



ST-2



UV-1



UV-2

TABLE VI-continued

## MULTILAYER FILM STRUCTURE



The preceding examples are set forth to illustrate specific embodiments of this invention and are not intended to limit the scope of the compositions, materials or methods of the invention. Additional embodiments and advantages within the scope of the claimed invention will be apparent to one skilled in the art.

What is claimed is:

1. A photographic element, comprising a support bearing at least one silver halide emulsion and at least one 3-indoloylacetanilide yellow dye-forming coupler of structure I, below:



wherein:

R<sub>1</sub> is an alkyl or phenyl group;

R<sub>2</sub> is a phenyl, t-butyl, cyclohexyl or naphthyl group;

X is a halogen atom or an alkoxy or alkyl group;

each R<sub>3</sub> is in the para position or either meta position relative to the anilino nitrogen and is individually selected from the group consisting of halogen atoms, and alkyl, phenyl, alkoxy, phenoxy, carbamoyl, sulfamoyl, carbonamido, sulfonamido, alkylsulfonyl, arylsulfonyl, alkoxy carbonyl, aryloxycarbonyl, acyloxy, sulfoxy, sulfonyloxy, alkylthio, acyl and cyano groups;

n is 1, 2 or 3;

R<sub>4</sub> is a hydrogen atom or an alkyl group;

R<sub>5</sub> is a hydrogen atom or an alkyl group; and

each R<sub>6</sub> is individually a halogen atom, an alkyl group or an alkoxy group and m is 0-4;

provided that substituents may join to form a ring.

2. A photographic element according to claim 1, wherein the 3-indoloylacetanilide coupler is coated in the same layer with at least one blue sensitive silver halide emulsion.

3. A photographic element according to claim 2, wherein the blue sensitive silver halide emulsion is a tabular grain emulsion.

4. A photographic element according to claim 1, wherein R<sub>2</sub> is a phenyl group.

5. A photographic element according to claim 1, wherein R<sub>1</sub> is an alkyl group.

6. A photographic element according to claim 1, wherein X is a halogen atom.

7. A photographic element according to claim 1, wherein n is 1 and R<sub>3</sub> is a carbamoyl group or a sulfamoyl group in either the 4- or 5-position relative to the anilino nitrogen.

8. A photographic element according to claim 1, wherein at least one of R<sub>4</sub> and R<sub>5</sub> is an alkyl group.

9. A photographic element according to claim 1, wherein R<sub>4</sub> and R<sub>5</sub> are alkyl groups.

10. A photographic element according to claim 9, wherein both R<sub>4</sub> and R<sub>5</sub> are methyl groups.

11. A photographic element according to claim 1, wherein m is 0.

12. A photographic element according to claim 1, wherein coupler I is coated at a level between 0.05 and 3.00 g/sq m.

13. A photographic element according to claim 1, wherein coupler I is selected from the group consisting of:

A1



A2



A3



A4



A5





and



**14.** A photographic element according to claim **1**, wherein an imaging coupler of claim **1** is coated in the same layer as a yellow dye-forming DIR coupler.

**15.** A method for providing a thermally stable photographic image comprising processing of a photographic element according to claim **1** in a color developer solution.